

## UNITED STATES PATENT OFFICE

2,329,575

## PROPELLENT POWDER

Elton R. Allison, Wharton, and Ellsworth S. Good-year, Kenilworth, N. J., assignors to Hercules Powder Company, Wilmington, Del., a corporation of Delaware

No Drawing. Application July 30, 1940,  
Serial No. 348,552

5 Claims. (Cl. 52—20)

This invention relates to an improved propellant smokeless powder and more particularly to a novel and improved method of producing a high gravimetric density, free flowing, non-clustering, progressive burning smokeless powder.

Heretofore the art has recognized and used surface coated propellant powder. The surface coated propellant powder which the art produced by coating powder grains with a deterrent material have proved partially satisfactory but there are a number of disadvantages to the known processes of coating. The powder grains coated with deterrent materials by the accepted processes now known to the art are not entirely successful because in all instances there is a tendency for the individual grains to be coated with unequal amounts of deterrent. Unequal coating results in clustering, low gravimetric densities and non-uniform ballistics.

The basic methods of coating smokeless powder with deterrent materials now used by the art comprises, in general, the tumbling or stirring of powder grains in the presence of a quantity of deterrent material. The tumbling or stirring process is normally carried out in a revolving drum or "sweetie barrel" and the coating processes now used are aided by the addition to the drum of solvents or non-solvents for the powder grains and coating materials such as is more particularly described in U. S. Patents 1,661,278 to Troxler; 2,113,418 to Woodbridge; 2,152,509 to Troxler; 2,028,990 to Olsen; 1,955,927 to McBride; and 1,967,913 to Tibbets.

Each of the above methods described in the foregoing prior art patents produces propellant smokeless powder grains which finally receive a coating of deterrent material which is not substantially equally deposited on all surfaces of the grains and which therefore are not of the highest gravimetric density nor of the uniform ballistics required by modern high velocity rifles and guns. The smokeless powder by the prior art methods was found to be more or less sticky, tended to form clusters and did not load freely into cartridge shells. The non-free flowing disadvantage is mainly due to the lack of a uniform coating of deterrent material on the surface of the grains. Manufactured powders, due to the above difficulties often fail to test satisfactory and have to be reworked with consequent loss of time and production.

It is the object of this invention to provide means whereby deterrent substances present on the surface of coated smokeless powder grains

may be evenly distributed on the surface of said smokeless powder grains.

A further object of this invention is to provide a coated smokeless powder having a high gravimetric density and free loading characteristics.

A further object is to provide a method of redistributing an uneven coating of deterrent material.

A still further object of this invention is to provide a smokeless powder of improved ballistics, quality and regularity. Other objects of this invention will appear hereinafter.

In general, the objects of this invention are accomplished by treating surface coated smokeless powder produced under methods well known in the art, by an additional step which redistributes the deterrent coating on the grain surface in such a manner that a substantially equal coating of the deterrent material is obtained on all surfaces of each grain. The additional step includes the treatment of the coated smokeless powder grains with a volatile liquid which is a non-solvent or a poor solvent for the powder grains themselves, but which is a weak solvent for the deterrent material used as a coating for the powder grains.

More specifically the treatment in accordance with this invention comprises placing a charge of surface coated powder grains into a sweetie barrel and adding thereto about 6 to 10% by weight of a volatile liquid which is substantially a non-solvent for the powder grains and which is a very weak solvent for the deterrent thereon. Usually ethyl alcohol or admixtures thereof with water will be found desirable as the volatile liquid depending upon the deterrent to be redistributed. The powder charge within the sweetie barrel is heated by means of a water bath to between about 10° C. and about 20° C. below the boiling point of the volatile liquid and then tumbled for between about 15 minutes and two hours or until the volatile liquid has redissolved and redistributed the deterrent coating originally on the grains into a substantially equal layer of deterrent coating over the entire surface of each grain.

It is thought that the volatile liquid redistributes the deterrent material by dissolving it from those surfaces of the powder grains having a high concentration of the deterrent material and depositing it on those surfaces having a low concentration of the deterrent material until an equilibrium may be reached wherein there is equal concentration of the deterrent material on all surfaces, however, the treatment with the volatile vehicle may increase the penetration. The

redistribution or penetration of the deterrent material effected eliminates stickiness of the powder grain and the resulting powder flows more freely, has a higher density, and gives better ballistics than powder not given the treatment. The volatile vehicle preferred for use is 95% ethyl alcohol diluted with from about 20% to about 50% water. The vehicle should be selected so that from about 5% to about 50% of the deterrent material present on the grains may be dissolved therein.

The treatment in accordance with this invention may be carried out in the sweetie barrel directly after the coating and so doing the water present in the powder is used to dilute the alcohol.

The powder is heated at a temperature near the melting point of the deterrent material for from 15 minutes to two hours, depending upon how much redistribution of the deterrent material is necessary. Although an alcohol-water mixture containing from 70-80% alcohol is preferably used, mixtures containing 50-95% alcohol can be used. However the treatment is also specifically adapted for treatment of coated powders which have been completed and found by ballistic tests to be unsatisfactory.

Other volatile liquids which have been found adaptable for the procedure in accordance with this invention are those liquids similar in action to ethyl alcohol and ethyl alcohol-water mixtures mentioned above such as, for example, dioxane, acetone, petroleum naphtha, butyl acetate and the like, either alone or in admixture with each other or with water. Mixtures of dioxane and water, acetone and water, petroleum naphtha and butyl acetate have been found especially desirable. The volatile liquids which are to be used for the process of this invention should have a boiling point less than that of water and in no instance higher than about 120° C. as the treatment of the powder grains above about 80 to 90° C. may cause decomposition and affect the stability of the powder.

The actual redistribution procedure of this invention is carried out by the addition of the so-called volatile liquid to a given weight of coated propellant powder grains and the grains and liquid tumbled in a sweetie barrel for a period of time and at a temperature sufficient to cause the liquid to act as a solvent for the coating and to cause the liquid to evaporate thus leaving the coating evenly distributed on the surface of the individual powder grains.

In order to specifically point out the improvement which is obtained by the method of my invention, the following progressive burning propellant smokeless powders were prepared:

#### EXAMPLE 1

A double base tubular rifle powder, granulated .070 x .015 x .091 and containing 20% nitroglycerin was coated with ethyl ortho benzoyl benzoate by the coating method described in U. S. Patent 2,152,509. The procedure following comprised the addition of 4 parts by weight of water to 50 parts by weight of powder grains contained in a sweetie barrel. The barrel was revolved, and to the water wet powder 1.25 parts by weight of ethyl ortho benzoyl benzoate was added. The barrel was covered and tumbled for 45 minutes at a water bath temperature of 65° C., after which two parts by weight of additional water and .875 part by weight of additional ethyl ortho benzoyl benzoate were added. The barrel was revolved for an additional 50 minutes at 65° C. and then 2 parts of additional water and

.625 part of additional parts of ethyl ortho benzoyl benzoate were added. The barrel was revolved an additional 30 minutes at 65° C., then 15 minutes without the application of heat. After the cooling period, the powder was dried for one day at 55° C., glazed with graphite, screened to remove the fine and coarse powder, humidified by exposure to 60% relative humidity and then tested for ballistics and gravimetric density. The above powder is classed as coated powder and is a commercial powder known to the art. The powder had a gravimetric density of .900 and when tested in a .50 caliber rifle allowed a charge of 202 grains to be inserted in the cartridge which gave a velocity of 2670 ft. per second, and a pressure of 49,000 lbs. per sq. inch.

#### EXAMPLE 2

A portion of the coated powder as described in the Example 1 above was treated in accordance with this invention by placing 1812 parts by weight of the powder in a sweetie barrel, adding thereto 180 parts by weight of ethyl alcohol and about 20 parts by weight of water and revolving the barrel for about one hour at a temperature of 65° C. The barrel was revolved an additional 15 minutes without the application of heat after which the powder was dried for a day at 55° C., glazed with graphite, screened to remove the fine and coarse powder, humidified by exposure to 60% relative humidity and then tested for ballistics and gravimetric density in the same manner as the powder of Example 1 was tested. The powder of this example has a gravimetric density of .995 and when tested in a .50 caliber rifle allowed a charge of 241 grains of powder to be placed in the cartridge which gave a velocity of 2888 ft. per second and a pressure of 48,000 lbs. per sq. inch.

A comparison of the results obtained with coated powder manufactured by a prior art method (Example 1) and the results obtained with a coated powder treated in accordance with this invention (Example 2) shows that the process of this invention increased the gravimetric density of the powder grains by .095 which allowed an increase in charge of 39 grains, which increased the velocity of the bullet by 218 ft. per second, while decreasing the pressure of 1000 lbs. per sq. in. These results indicate that a great improvement is made by giving coated powder the treatment of this invention.

To further show the improvement effected when coated powder grains are treated by the process of this invention, the following examples are given and the results of gravimetric density and ballistics are listed in Table I.

#### EXAMPLE 3

1812 parts by weight of coated grains described in Example 1 were placed in a sweetie barrel and tumbled at 65° C. with 145 parts by weight of alcohol and 36 parts by weight of water. After this operation the powder grains were cooled, glazed, screened, humidified, and tested in the manner described in Examples 1 and 2.

#### EXAMPLE 4

The coated grains prepared in Example 1 were given the same treatment as described in Example 3 except that the temperature of treatment was 40° C.

#### EXAMPLE 5

The coated grains prepared in Example 1 were

given the same treatment as described in Example 3 except that the temperature of treatment was 85° C.

EXAMPLE 6

1812 parts by weight of coated grains described in Example 1, were placed in a sweetie barrel and tumbled at 65° C. with 72 parts by weight of alcohol and 36 parts by weight of water. After this operation the powder grains were cooled, glazed, screened, humidified and tested in the manner described in Examples 1 and 2.

EXAMPLE 7

A sample of powder was treated in the same way as described in Example 6 except that 75 parts by weight of alcohol and 36 parts by weight of water were used.

EXAMPLE 8

A sample of powder was treated in the same way as described in Example 6 except that 360 parts by weight of alcohol and 90 parts by weight of water were used.

The results of testing the above powders are given in Table I:

Table I

| Example | Gravimetric density | Charge | Velocity | Pressure |
|---------|---------------------|--------|----------|----------|
| 1       | .900                | 202.0  | 2,670    | 49,000   |
| 2       | .995                | 241.0  | 2,888    | 48,000   |
| 3       | .989                |        |          |          |
| 4       | .956                | 220.0  | 2,752    | 48,000   |
| 5       | .993                |        |          |          |
| 6       | .967                | 224.0  | 2,776    | 47,600   |
| 7       | .982                |        |          |          |
| 8       | .974                |        |          |          |

EXAMPLE 9

As a further example, a sample of prior art powder was manufactured and coated with dinitrotoluene. The coating process comprised adding 1812 parts by weight of rifle powder containing 20% nitroglycerin to a sweetie barrel, wetting the powder with 125 parts by weight of water and sprinkling thereon 190 parts by weight of dinitrotoluene. The barrel was then revolved for 40 minutes at a temperature of 85° C. After this treatment, 145 parts of additional water and 90 parts of additional dinitrotoluene were added and the barrel revolved 1 hour at 85° C.

One-half of the above coated powder was cooled, dried, glazed, screened, and humidified and then submitted to ballistic and gravimetric density testing. The other half of the still wet coated powder was treated in accordance with this invention by placing it back in the sweetie barrel, adding 90 parts by weight of alcohol and revolving the barrel for one hour at 85° C. This treated sample was cooled, glazed, screened, humidified and then tested for gravimetric density and ballistics. The comparative results of the two powders are given in Table II:

Table II

| Example 9     | Gravimetric density |
|---------------|---------------------|
| Coated grain  | .957                |
| Treated grain | .984                |

From the above table, it is noted that the gravimetric density of the treated grains has been materially increased.

EXAMPLE 10

As a further example of my invention, a .50 caliber powder having a granulation of .070 x .015 x .091 was coated as follows: 550 parts by weight of powder were wet with 40 parts by weight water, and 16 parts by weight Centralite (symmetrical diethyl diphenylurea) were added and the barrel revolved for 45 minutes at 87° C. To the powder was then added 20 parts additional water and 9 parts additional Centralite and the barrel revolved for 45 minutes at 87° C. After this treatment, 20 parts by weight additional water and 5 1/2 parts by weight of additional Centralite were added and the sweetie barrel revolved for 30 minutes at 87° C. In this manner, a total of 7,000 lbs. of .50 caliber powder was coated so that the coating of the Centralite varied between 5 1/4 to 6%. The powder was dried, glazed, screened and humidified and then had a gravimetric density of .952, and a charge of 232 grains of the powder gave a velocity of 2832 ft. per second and a pressure of 51,000 lbs. per sq. inch in a .50 caliber rifle.

EXAMPLE 11

A portion of powder prepared as described above was then treated in accordance with this invention by placing it in a sweetie barrel and adding 10% by weight of an alcohol-water (80-20) mixture. After treatment by revolving the barrel for 15 minutes at 50° C. and 45 minutes at 60° C., the powder was dried, glazed, screened, and humidified and when tested gave a gravimetric density of .979 in a .50 caliber rifle. A charge of 240 grains gave a velocity of 2905 ft. per second with a pressure of 48,900 lbs. per sq. inch. A comparison of the above figures shows that the treatment in accordance with this invention increases the gravimetric density of powder grains and provides better ballistics in given components.

EXAMPLE 12

In order to further show the improved results of this invention 50 parts by weight of .50 caliber double base powder having a granulation of .070 x .015 x .091 were placed in a sweetie barrel and wet with 3.5 parts by weight of water and 1 part by weight of Centralite #1 (symmetrical diethyl diphenyl urea) were added and the barrel revolved for 45 minutes at 85° C. To the powder was then added 1.75 parts by weight of additional water and 0.875 part by weight additional Centralite #1 and the barrel revolved for 45 minutes at 85° C. After this treatment, 1.75 parts by weight additional water and 0.75 part by weight additional Centralite were added and the barrel revolved for 30 minutes at 85° C. After this treatment the barrel was revolved for 15 minutes without further heating and the powder then removed from the barrel, dried, glazed, screened, and humidified. This powder designated as coated untreated powder is compared with treated samples in Table III which will follow.

EXAMPLE 13

A portion of the coated powder prepared as described above was further treated in accordance with this invention by placing it in a sweetie barrel and adding 10% by weight of an 80-20 dioxane-water mixture. After treatment by revolving the barrel for 15 minutes at 50° C. and then for 45 minutes at 60° C. the powder was dried, glazed, screened, and humidified. This powder

is designated coated dioxane-water treated powder in Table III.

EXAMPLE 14

Another portion of the coated untreated powder described above was further treated in accordance with this invention by placing it in a sweetie barrel and adding 10% by weight of 30-70 acetone-water mixture. Other details of the treatment were exactly as described in the previous example. The finished powder is designated as coated acetone-water treated powder in Table III.

EXAMPLE 15

Another portion of the coated untreated powder described above was further treated in accordance with this invention by placing it in a sweetie barrel and adding 10% by weight of a 90-10 petroleum naphtha-butyl acetate mixture. Other details of the treatment were exactly as described in the previous example. The finished powder is designated as coated petroleum naphtha-butyl acetate treated powder in Table III.

The coated untreated powder and the three coated treated powders were tested for gravimetric density and ballistics in a .50 Ca. rifle. The comparative results obtained with the different powders are given in Table III below.

TABLE III

| Treatment type                       | Gravimetric density | Charge gr. | Velocity f.s. | Pressure lbs./sq. in. |
|--------------------------------------|---------------------|------------|---------------|-----------------------|
| None.....                            | .928                | 220        | 2,899         | 50,600                |
| Dioxane-water.....                   | .983                | 250        | 3,051         | 49,400                |
| Acetone-water.....                   | .971                | 226        | 2,932         | 50,000                |
| Petroleum-naphtha-Butyl-acetate..... | .948                | 225        | 2,927         | 50,100                |

From the above table it is noted that the gravimetric density of the treated samples has been increased and that the deterrent action of the coating has been made more effective as is shown by the ability to load the treated powders to higher velocities without exceeding the pressure obtained with the coated untreated powder.

The treatment in accordance with this invention gives high yields of unclustered grains and at the same time gives a smokeless powder which is of highest quality and which is better ballistically than the powders manufactured by prior art methods.

It will be understood that the details and examples hereinbefore set forth are illustrative only, and that the invention as broadly described and claimed is in no way limited thereby.

What we claim and desire to protect by Letters Patent is:

1. A process for producing improved progressive-burning surface-modified propellant smokeless powder grains which includes the steps of placing progressive burning smokeless powder grains having a coating of deterrent material on their surfaces into tumbling means, adding thereto a volatile liquid which is a non-solvent for

the said grains but is a weak solvent for the said deterrent on the said grains, heating the solvent and grains to a temperature substantially below the boiling point of the volatile liquid and tumbling the grains, whereby the said deterrent is redistributed and deposited on all surfaces of the said grains in a substantially equal coating.

2. A process for producing improved progressive-burning surface-modified propellant smokeless powder grains which includes the steps of adding to smokeless powder grains, having deposited on their surface a deterrent material, a volatile liquid which is a non-solvent for said grains but which is a weak solvent for said deterrent, heating the liquid wet grains to a temperature substantially below the boiling point of the liquid, and tumbling said grains and liquid, whereby the said deterrent is redistributed and deposited on all surfaces of the said grains in a substantially equal coating.

3. A process for producing improved progressive-burning surface-modified propellant smokeless powder grains which includes the steps of adding to smokeless powder grains, having deposited on their surface the deterrent symmetrical diethyl diphenyl urea, an alcohol water mixture, which is a non-solvent for said grains but which is a weak solvent for said deterrent heating the alcohol water wet grains to between about 10° C. and about 20° C. below the boiling point of the alcohol water mixture and tumbling said grains and liquid, whereby the said deterrent is redistributed and deposited on all surfaces of the said grains in a substantially equal coating.

35 4. A process for producing improved progressive-burning surface-modified propellant smokeless powder grains, which includes the steps of adding to smokeless powder grains, having deposited on their surface the deterrent dinitrotoluene, an alcohol water mixture which is a non-solvent for said grains but which is a weak solvent for said deterrent heating the alcohol water wet grains to between about 10° C. and about 20° C. below the boiling point of the alcohol water mixture and tumbling said grains and liquid, whereby the said deterrent is redistributed and deposited on all surfaces of the said grains in a substantially equal coating.

40 5. A process for producing improved progressive-burning surface-modified propellant smokeless powder grains which includes the steps of adding to smokeless powder grains, having deposited on their surface the deterrent ethyl ortho benzoyl benzoate, an alcohol water mixture, which is a non-solvent for said grains but which is a weak solvent for said deterrent heating the alcohol water wet grains to between about 10° C. and about 20° C. below the boiling point of the alcohol water mixture and tumbling said grains and liquid, whereby the said deterrent is redistributed and deposited on all surfaces of the said grains in a substantially equal coating.

ELTON R. ALLISON.

ELLSWORTH S. GOODYEAR.